

# UNITED STATES PATENT OFFICE.

GOTTFRIED DIESSER, OF ZURICH, SWITZERLAND.

## PROCESS FOR MAKING SILK FELTABLE.

1,156,983.

Specification of Letters Patent.

Patented Oct. 19, 1915.

No Drawing.

Application filed May 20, 1914. Serial No. 839,864.

*To all whom it may concern:*

Be it known that I, GOTTFRIED DIESSER, a subject of the Emperor of Germany, residing at Zurich, Switzerland, have invented 5 new and useful Improvements in Processes for Making Silk Feltable; and I do hereby declare the following to be a full, clear, and exact description of the invention, such as will enable others skilled in the art to which 10 it appertains to make and use the same.

The manufacture of felt is based on the property of certain fibrous materials to felt, that is to entangle in such a close manner under certain conditions that a compact 15 body of great toughness is produced.

The process according to this invention depends on the albuminous character of the silk and on the absorbent properties of the latter and also on the property of the silk 20 to partly dissolve in cold formic acid, without a further cleaving of the molecule of fibroin taking place.

According to one convenient mode of carrying this invention into effect the short 25 fibrous silk (waste-silk) is freed in a well known manner from the bast and then treated with cold water until the fiber is well washed. Hereupon the silk is washed with formic acid until a fibrous pulp of 30 uniform quality is obtained and this pulp is then put in suitable sieves, so that the formic acid can run off. The fibrous cake is then finally dried. Thus a very tough 35 body is obtained, which has at first a paper-like appearance and which after having been treated in suitable machines may then be converted into a felt-like body.

According to a second convenient mode of carrying this invention into effect the silk is at first freed in a well known manner from the bast and the material is then well washed out and treated in water until a fibrous pulp of uniform quality is obtained. Suitable provisions are then made for removing the excess of water and the pulp 40 cake is hereupon dried and exposed to the 45 action of gaseous formic acid.

In both cases the silk fiber is superficially dissolved by the formic acid, the degree of the solution depending upon the time during 50 which said acid acts upon the fiber. During the volatilization of the formic acid the original solution of fibroin sticks together 55 the single fibers in an extraordinarily strong manner. As the silk material is insoluble in water, the solution of the fibroin in formic acid will also deliver products, which are insoluble in water and the resulting silk-felt will therefore form a material, which cannot be dissolved by water. 60

What I claim is:

A process for making silk capable of being felted, consisting in exposing the silk to the action of liquid or gaseous formic acid to form a fibrous pulp and subsequently 65 drying the silk.

In testimony that I claim the foregoing as my invention I have signed my name in presence of two subscribing witnesses.

GOTTFRIED DIESSER.

Witnesses:

CARL SUEWER,  
ARNOLD LEHUE.